



US012460325B2

(12) **United States Patent**  
**Atil et al.**

(10) **Patent No.:** US 12,460,325 B2  
(45) **Date of Patent:** Nov. 4, 2025

(54) **WOVEN FURRY FABRIC AND A METHOD OF PRODUCTION THEREOF**

(71) Applicant: **Sanko Tekstil Isletmeleri San. Ve Tic. A.S.**, Inegol-Bursa (AR)

(72) Inventors: **Ezgi Atil**, Inegol-Bursa (AR); **Erdogan Baris Ozden**, Inegol-Bursa (AR)

(73) Assignee: **Sanko Tekstil Isletmeleri San. Ve Tic. A.S.**, Inegol-Bursa (TR)

(\*) Notice: Subject to any disclaimer, the term of this patent is extended or adjusted under 35 U.S.C. 154(b) by 135 days.

(21) Appl. No.: **16/830,168**

(22) Filed: **Mar. 25, 2020**

(65) **Prior Publication Data**

US 2020/0308731 A1 Oct. 1, 2020

(30) **Foreign Application Priority Data**

Mar. 26, 2019 (EP) ..... 19165322

(51) **Int. Cl.**

**D03D 13/00** (2006.01)  
**D02G 3/02** (2006.01)  
**D02G 3/44** (2006.01)  
**D03D 1/00** (2006.01)  
**D03D 15/54** (2021.01)

(52) **U.S. Cl.**

CPC ..... **D03D 13/004** (2013.01); **D02G 3/02** (2013.01); **D02G 3/44** (2013.01); **D03D 15/54** (2021.01); **D03D 1/00** (2013.01)

(58) **Field of Classification Search**

None

See application file for complete search history.

(56)

**References Cited**

U.S. PATENT DOCUMENTS

6,799,581 B2 \* 10/2004 Cave ..... A45D 8/34  
132/273  
7,188,642 B2 \* 3/2007 James ..... G02B 6/4459  
139/384 R  
7,300,692 B2 \* 11/2007 Hirota ..... D03D 27/06  
428/92

(Continued)

FOREIGN PATENT DOCUMENTS

EP 3205755 A1 \* 8/2017 ..... D01D 5/30  
JP 2002061070 A \* 2/2002

(Continued)

OTHER PUBLICATIONS

Choudhury, Asim Kumar Roy. "Indigo Dye: Various Ecofriendly Finishes 14.3.8 Denim Biowash." Indigo Dye—an Overview | Science Direct Topics, Principles of Textile Finishing, 2017, <https://doi.org/10.1016/B978-0-08-100646-7.00014-X>. (Year: 2017).\*

(Continued)

*Primary Examiner* — Grace Huang

(57) **ABSTRACT**

A furry fabric includes a woven fabric having a plurality of warp and/or weft yarns extending over a number of weft or warp yarns and/or below a number of weft or warp yarns to provide over and/or under-portions having a length comprised between 8 and 3000, preferably between 25-3000. The over and under portions are at least in part cut in a garment including the furry fabric. Alternatively, the warp or weft over portions and/or the warp or weft under portions of said first yarns are not cut or broken.

**27 Claims, 14 Drawing Sheets**



|                       |                         |         |                        |  |  |
|-----------------------|-------------------------|---------|------------------------|--|--|
| (56)                  | <b>References Cited</b> |         |                        |  |  |
| U.S. PATENT DOCUMENTS |                         |         |                        |  |  |
| 139/383 R             |                         |         |                        |  |  |
| 7,571,746             | B2 *                    | 8/2009  | Hay .....              |  |  |
| 9,365,958             | B2 *                    | 6/2016  | Yenici .....           |  |  |
| 9,885,130             | B2 *                    | 2/2018  | Yenici .....           |  |  |
| 10,051,905            | B2 *                    | 8/2018  | Benefiel .....         |  |  |
| 10,104,917            | B2 *                    | 10/2018 | Liao .....             |  |  |
| 10,167,579            | B2 *                    | 1/2019  | Kilickan .....         |  |  |
| 10,221,506            | B2 *                    | 3/2019  | Yenici .....           |  |  |
| 10,378,127            | B2 *                    | 8/2019  | Aydelette .....        |  |  |
| 11,021,814            | B2 *                    | 6/2021  | Kilickan .....         |  |  |
| 11,208,761            | B2 *                    | 12/2021 | St. Onge-Simpson ..... |  |  |
|                       |                         |         | B23K 26/0006           |  |  |
| 11,241,055            | B2 *                    | 2/2022  | Love .....             |  |  |
| 11,572,641            | B2 *                    | 2/2023  | Yenici .....           |  |  |
| 12,024,800            | B2 *                    | 7/2024  | Kalfa Kilickan .....   |  |  |
| 2012/0278981          | A1 *                    | 11/2012 | Ialenti .....          |  |  |
|                       |                         |         | A41B 11/02             |  |  |
|                       |                         |         | 2/24                   |  |  |
| 2013/0115841          | A1 *                    | 5/2013  | Ronner .....           |  |  |
|                       |                         |         | D03D 15/258            |  |  |
|                       |                         |         | 28/165                 |  |  |

|              |      |        |                      |              |
|--------------|------|--------|----------------------|--------------|
| 2016/0083877 | A1 * | 3/2016 | Kalfa Kilickan ..... | B32B 7/12    |
|              |      |        |                      | 156/60       |
| 2017/0233904 | A1 * | 8/2017 | Weening .....        | D03D 13/00   |
|              |      |        |                      | 139/420 R    |
| 2019/0151494 | A1 * | 5/2019 | Selva Sarzo .....    | A61F 13/0273 |

## FOREIGN PATENT DOCUMENTS

|    |               |   |        |
|----|---------------|---|--------|
| JP | 2008031583 A  | * | 2/2008 |
| WO | 2011104022 A1 |   | 9/2011 |

## OTHER PUBLICATIONS

“Sodium Bisulfate: Common Names, Compound Name and More.”  
 Jones Hamilton. Jul. 4, 2022. <http://web.archive.org/web/20220704234804/https://www.jones-hamilton.com/sodium-bisulfate-compound-names/> (Year: 2022).\*

European Search Report issued by the EPO on Sep. 30, 2019 for corresponding EP application No. 19165322.9.

International Search Report issued by the EPO on Jun. 30, 2020 for corresponding PCT application No. PCT/EP2020/058467.

\* cited by examiner



FIG.1



FIG.2



FIG.3



FIG. 4



FIG.5



FIG. 6



FIG. 7



FIG. 8



FIG.9



FIG. 10



FIG.11



FIG.12



FIG.13



**FIG.14**



**FIG.15**



FIG.16

## 1

WOVEN FURRY FABRIC AND A METHOD  
OF PRODUCTION THEREOF

This application claims priority to and the benefit of European Application No. 19165322.9 filed on 26 Mar. 2019, the content of which is incorporated herein by reference in its entirety.

## TECHNICAL FIELD

The technical field of the present invention relates to a woven fabric that imitates natural fur, i.e. has a furry appearance, and to a method of producing such fabric.

In particular, the present invention relates to a woven fabric that is used to produce clothing articles and garments. A preferred type of fabric of the invention is a denim fabric or a fabric having a denim look; in a preferred embodiment at least part of the yarns are indigo dyed. Denim is referred to in the following description, but the invention is not limited to the production of denim fabrics only.

The invention comprises also a method of production of a woven fabric having a furry appearance as above mentioned.

## BACKGROUND

Fabrics that imitate animal furs have been known for a long time. For example, GB3015, filed on 5 Feb. 1914 in the name of Hammer, discloses a fabric that is woven double in the loom and that is divided to provide a fur imitation fabric. Another fur imitation fabric is disclosed in U.S. Pat. No. 5,609,935; this document teaches to manufacture a pile fabric out of different polyester fibers. The two types of polyester fibers protruding from the base fabric have different resistance to alkali so that the less alkali-resistant fibers can be shortened by an alkali agent to better imitate a natural fur.

A fabric having a furry appearance can also be created using specialized knitting or weaving machines which are not common for denim production. Another option is to use a highly specialized manual manufacturing process which is expensive and needs long production times and cannot easily be adapted to industrial production in high volumes. There is therefore the need of providing an improved fabric that imitates fur, i.e. has a furry appearance, and method of producing the same in an economic way that is simple to implement on existing looms and weaving machines.

An aim of the invention is to solve the above problems and to provide a woven fabric imitating fur that is created using common machines such as dobby machines or jacquard machines using particularly designed weaving reports.

Denim is a popular fabric that is produced by weaving weft and warp yarns in a twill design. Weaves that are employed for denim manufacture vary depending on the area of application. Fine denim fabrics are normally composed of plain weaves. However, denim fabrics that are conventionally used under slightly rougher conditions are made using a twill weave, namely a weave characterized by a diagonal pattern.

A further aim of the invention is thus to provide a woven fabric, including indigo dyed fabrics, having a furry appearance and suitable to give a general appearance of fur, i.e. a furry appearance while providing at the same time a look that reminds the user of indigo denim. In other words, it is an aim of the invention to provide a fabric, and eventually

## 2

a garment, that has a fur look and that is obtained from a woven fabric produced with commonly available machines by an inexpensive method.

This and other aims are achieved by a woven fabric according to claim 1 and by a method according to claim 10. The dependent claims delineate preferred and/or especially advantageous aspects. The invention also relates to a garment according to claim 16.

## 10 SUMMARY OF THE INVENTION

An embodiment of the invention provides a woven fabric having a fur-like look, the woven fabric having warp yarns and weft yarns, said fabric having a front side and a back side, said warp and weft yarns being woven together in a weaving pattern, the weaving pattern comprising a base and at least one of warp or weft over portions and/or at least one of warp or weft under portions, whereby at least one of the warp or weft yarns are extending over a number of weft or warp 15 yarns and below a number of weft or warp yarns to provide said warp or weft over portions in said front side and/or warp or weft under portions in said back side and wherein the warp over portions or the warp under portions are long, i.e. they have a length comprised between 8 and 20 3000 yarns. Similarly, the weft over portions or the weft under portions are long, i.e. they have a length comprised between 25 and 3000 25 yarns.

An advantage of this embodiment is that it makes possible to have very long over portions on the warp side or on the weft side, namely on the front side of the fabric, such over portion being suitable for creating a furry appearance to the final product without requiring any special machine or process.

The invention further comprises a method of preparing a 30 fabric according to claim 10. The method includes the steps of weaving warp yarns or weft yarns following a pattern comprising a base and warp or weft over portions and/or warp or weft under portions, whereby said warp and weft 35 yarns are woven together in a weaving pattern, the weaving pattern comprising a structural base of the fabric and at least one of warp or weft over portions and/or at least one of warp or weft under portions, whereby at least one of the warp or weft 40 yarns are extending over a number of weft or warp yarns and below a number of weft or warp yarns to provide said warp or weft over portions in said front side and/or warp or weft under portions in said back side and wherein the warp over portions or the warp under portions have a length comprised between 8 and 3000 45 yarns, preferably 8-300 50 yarns and the weft over portions or the weft under portions have a length comprised between 25 and 3000 55 yarns, preferably 25-300 60 yarns. Preferably, the warp and/or weft over or under portions have a length of 30 to 450 65 yarns, more preferably of 40 or 45 to 400 70 yarns. According to another embodiment, the fabric is provided with warp over portions or warp under portions (or both) having a length of 30 to 450 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410 9415 9420 9425 9430 9435 9440 9445 9450 9455 9460 9465 9470 9475 9480 9485 9490 9495 9500 9505 9510 9515 9520 9525 9530 9535 9540 9545 9550 9555 9560 9565 9570 9575 9580 9585 9590 9595 9600 9605

side of the fabric; a garment obtained from the fabric of this embodiment will be provided with the long over portions at least (possibly only) on the front side of the garment, i.e. the visible side of the garment. The back of the fabric is the side intended to be in contact with the wearer's body. According to an embodiment at least the warp yarns provided with the said long over portions (on the front side) are dyed, more preferably ring dyed; a suitable dye is black, indigo or another indigoid dye. The fabrics may also be a white fabric ready for dyeing or ecru fabric or any suitable color.

The fabric of the invention has alternated first and second warp yarns or first and second weft yarns or both. The first yarns, i.e. the first warp and/or weft yarns, have long over portions or under portions. The first yarns may have long over portions and long under portions; the long over portions and under portions may be provided in a same first yarn. These yarns provide the part of the fabric that imitates a fur, i.e. that gives a furry look to the garment. The second yarns have short over and under portions, e.g. portions floating, i.e. extending, over 1 to 3 or 4 yarns. The second yarns provide a base structure of the fabric. The base structure of the fabric is thus comprising a weaving of warps and wefts supporting the long over portions and under portions. It should be noticed that the fabric of the invention may have long over portions only warpwise; in such an embodiment the weft yarns are all second weft yarns, i.e. they concur to form a fabric base structure with the second warp yarns.

With the wording "alternated" it is meant that the first yarns are woven to be adjacent to one or more second yarns. Preferably the first and second yarns are alternated with a ratio "number of first yarns/number of second yarns" in the range 3/1 to 1/3, preferably 2/1 to 1/1. These arrangements are shown in the examples here below discussed.

According to an aspect of the invention, the length of the over portions in a same first yarn may be different. In this embodiment a yarn over portion may be e.g. long 20; the successive over portion may be long e.g. 15 and the following over portion may be long e.g. 30. The same may apply to the under portions of one yarn. Such feature may improve the natural look of the fabric. In an embodiment a feature that may provide a furry look to the fabric is the fact that the fabric may be woven with a twill arrangement. With "twill arrangement" it is meant that at least the second weft yarn floats across the second warp yarns in a progression of interlacings to the right or left, forming a pattern of distinct diagonal lines (a so-called wale).

Another feature that improves the fur look of the fabric is the fact that the over and under portions may have a discontinuity. According to another aspect of the invention, at least part of the long over portions or at least part of the long under portions or at least part of both in the first yarns have a discontinuity. In other words, the long portions of the first yarns are made of two portions that extend from the fabric base structure. The discontinuity is typically obtained by cutting the over/under portions. A suitable cutting means is a laser device for use in textiles.

In another embodiment, the over or under portions are broken or cut in any way which will be discussed more in detail in the following description. In another embodiment, the over or under portions are whole, i.e. they are not cut. In an embodiment, the warp long over portions are located on the front side of the fabric and are cut in two parts projecting from the fabric body; in this embodiment the back side of the fabric may have no long weft under portions or may have long weft under portions underportions that are whole, i.e. they are not cut.

The cutting process can be performed using any known cutting machine, even including the use of knife or may be obtained by the use of any type of suitable chemical treatment. Also laser cutting can be performed alternatively. It is possible to perform the cutting process on the fabric during the finishing process or it is possible to perform the cutting process on the garment or apparel obtained from the fabric. According to one embodiment, the cutting or breaking of the under or over portions is carried out before or during the washing treatment of the garment. Furthermore, chemical treatments for the fabric can be used for cutting and/or breaking the fibres. Possible chemical treatments are described in more detail in the following description.

It is an advantage of the present invention that an imitation fur fabric (and garment) may be obtained by using an inexpensive woven fabric having the claimed ranges of long over portions (and under portions). When the over portions in the finished fabric are cut, they curl in a fur-like look that may be further enhanced by additional treatments.

#### BRIEF DESCRIPTION OF THE DRAWINGS

Further aspects and advantages of the present invention will be discussed more in detail with reference to the enclosed drawings, given by way of non-limiting example, wherein:

FIG. 1 is a section view of a possible embodiment of the fabric according to the invention after weaving showing the over portions on the warp direction;

FIG. 2 is a section view of the fabric showing the over portions on the weft direction;

FIG. 3 is a weaving report, or scheme, of an embodiment of the fabric of the invention;

FIG. 4 is a weaving report of an alternative embodiment of the fabric of the invention;

FIG. 5 is a weaving report of still another embodiment of the fabric of the invention;

FIG. 6 is a weaving report in the weft direction of another embodiment of the fabric of the invention;

FIG. 7 is a further weaving report in the weft direction of another embodiment of the fabric of the invention;

FIG. 8 is still another weaving report in the weft direction of a further embodiment of the fabric of the invention;

FIG. 9 is another weaving report in the weft direction of a further embodiment of the fabric of the invention;

FIG. 10 is still another weaving report of a further embodiment of the fabric of the invention;

FIG. 11 is another weaving report of a further embodiment of the fabric of the invention;

FIG. 12 is a photograph of an embodiment of the fabric of the invention, illustrating the presence of over portions along the warp direction;

FIG. 13 is photograph an embodiment of the fabric of the invention illustrating the presence of over portions along the warp direction, the fabric being photographed after rinse wash;

FIG. 14 is a photograph of over portions on the weft direction.

FIG. 15 is photograph of an embodiment of the fabric of the invention after a cutting process; and

FIG. 16 is a flowchart of a method according to the invention.

#### DETAILED DESCRIPTION

Exemplary embodiments of the invention will now be described with reference to the enclosed drawings without intent to limit application and uses.

The invention will now be described with initial reference to FIG. 1 wherein a woven fabric **10** is depicted. The woven fabric **10** is obtained by crossing warp yarns w1, w2 and weft yarns 2, 2BS, 2FS, in a weaving pattern whereby the warp yarns w2 are extending over and below a number of weft yarns 2, 2BS, 2FS, to provide, with respect to the weft yarns 2, 2BS, 2FS, correspondent over portions and, eventually, under portions. Warp yarns w1 are interlaced with weft yarns 2, 2BS, 2FS, to provide a structural base portion of the fabric **10**.

In FIG. 1 under portions refer to portions being formed when warp yarns pass under a number of weft yarns 2, 2BS, 2FS, at the back side BS of the fabric, and over portions refer to portions of warp yarn w1, w2 that are formed when the warp yarns w1, w2 pass along the front side FS of the fabric and define connection portions. For example, the length of an over portion (or of an under portion) is measured by referring to the numbers of weft yarns 2, 2BS, 2FS, that is passed by the warp between two changes.

In many applications of the invention, the length of the over portions can be for the warp direction from 4 mm to 1400 mm, preferably 4-140 mm, most preferably 18 mm to 70 mm; for the weft direction from 8 mm to 1100 mm, preferably 8-110 mm, most preferably 12 mm to 50 mm.

FIG. 2 is a section view of a fabric according to another embodiment of the invention, globally indicated with the numerical reference **20**, showing over portions on the weft direction.

The woven fabric **20** is obtained by crossing weft yarns w'1, w'2 and warp yarns 2', BS', 2FS', in a weaving pattern whereby the weft yarns w'2 are extending over and below a number of warp yarns 2', BS', 2FS', to provide, with respect to the warp yarns 2', BS', 2FS' correspondent over portions and, eventually, under portions. Weft yarns w'1 are interlaced with warp yarns 2', BS', 2FS', to provide a structural base portion of the fabric **20**.

In FIG. 2 under portions refer to portions being formed when weft yarns pass under a number of warp yarns 2', BS', 2FS', at the back side BS' of fabric **20**, and over portions refer to portions of weft yarns w'2 that are formed when the weft yarns w'2 pass along the front side FS' of fabric **20** and define connection portions. For example, the length of an over portion (or of an under portion) is measured by referring to the numbers of warp yarns 2', BS', 2FS', that is passed by the weft between two changes.

In preferred embodiments of the invention, the warp over portions OP or the warp under portions have a length comprised between 8 and 3000 and the weft over portions OP' or the weft under portions have a length comprised between 25 and 3000.

As it is known, weave patterns can be conventionally displayed using weave symbols. In the present description, an integer number expressing a length such as the above mentioned numbers 8, 25 and 3000 indicates the count number of warp (or weft) yarns that are passed over (or under) by an over portion (or an under portion) of a weft (or warp) yarn, respectively.

In another embodiment, the warp or weft over portions (or under portions) have a length comprised between 30 to 450 yarns, preferably of 40 or 45 to 400 yarns more preferably in the range of 40 and 100 yarns.

The length in millimeters of the over portions can be for the warp direction from 4 mm to 1400 mm preferably 4 to 140 mm, more preferably, 18 mm to 70 mm; for the weft direction the length may be in the range of from 8 mm to 1100 mm, preferably 8 to 110 mm, more preferably 12 mm to 50 mm.

In an embodiment of the invention, for example, the fabric may be realized by using one warp yarn w2 for the mentioned over portions and the following warp yarn w1 is used for a regular weave pattern such as 1/1, 2/1 (such as the one depicted in FIGS. 1 and 2) or 3/1 and so on.

Alternatively, for example, two warp yarns w2 can be used for the over portions and a following warp w1 for a regular weave pattern to hold together the whole fabric construction therefore defining a base for the fabric. In 10 general, some warp yarns w2 are used to create the over portions and some warp yarns w1 are used in a regular weave pattern to hold together the fabric. The same is valid for fabric **20** of FIG. 2 in which warp yarns have been substituted with weft yarns and vice versa.

15 In this types of fabric, such as fabric **20**, therefore, some weft yarns w'2 are used to create the over portions and some weft yarns w'1 are used in a regular weave pattern to hold together the fabric forming a base for the fabric.

The fabric disclosed may be a standard rigid (non stretch) 20 fabric or, in a variant embodiment, it may be a stretch fabric or a bi-stretch fabric whereby at least some of the warp and/or weft or both warp and weft yarns are elastic.

Apart from indigo yarn dye or overdyed, the fabric disclosed may be black or white (ready for dyeing), ecru, or of 25 other colors, or of any overdyed color with different dye-stuffs such as sulphur dyes, reactive dyes, pigment, direct dyestuff. Also for the weft direction yarns may be black, overdyed or weft yarn dyed indigo.

30 Yarns of any fiber, natural or man-made can be used for the present invention. In particular, considering warp/weft yarns that are used for the base of the fabric, they may be from Ne 0.5 to Ne 400, most preferably Ne 7 to Ne 50. The warp or weft yarns used for the over portions may be from Ne 0.5 to Ne 400, preferably 0.5 to 40, more preferably Ne 2 to Ne 15 or Ne 4 to Ne 15. Warp numbers may be different 35 than each other or can be equal. Yarns may be one ply or multiply. Yarns can be any natural or man made fibres. Splittable yarns are not used in the present invention for the first warp or weft yarns, i.e. for the yarns provided with the 40 long over or under portions; preferably splittable yarns are not used at all. Suitable yarns, particularly for the first yarns, that provide the free-hanging portions of yarns and contribute to the visual effect, are metallized yarns. A yarn for the present invention may also be obtained by cutting a plurality 45 of stripes from a film, e.g. glittered stripes obtained from a glittered film. One yarn of this kind is e.g. known in the art and is commercially available from Lurex.

Some other examples of constructions may provide for 50 warp direction over portions of length from 4 mm to 1400 mm, preferably 4 to 140 mm, most preferably from 18 mm to 70 mm. For the weft direction the over portions may be long from 8 mm to 1100 mm, preferably 8-110 mm, most preferably from 12 mm to 50 mm.

FIG. 3 is a weaving report, or scheme, of an embodiment 55 of the fabric of the invention. FIG. 3 weaving report is a 12x84 construction representing the warp direction single front face fur design. For clarity such construction has been represented in two semi-reports, the construction of FIG. 3 being provided with a warp having a long (length is 79 weft 60 yarns) over portion and two short over portions (length 1) for odd-numbered warps and 28 over portions (of length 2) and 28 under portions (of length 1) for even numbered warps. The scheme is 79/1/1/1/1 (bottom to top) for odd-numbered warps and 2/1 for even numbered warps.

In the scheme of FIG. 3 the weft has two long under 65 portions (length 5) and two short over portions (length 1)

except for picks 10, 24, 38, 52, 66 and 80 where the weft has one under portion of length 5, two under portions of length 2 and three over portions of length 1 and therefore a scheme of 5/1/2/1/1/2/1.

Also for picks 12, 26, 40, 54, 68 and 82, the weft has one under portion of length 5, one under portion of length 4, one over portion of length 2 and one over portion of length 1, the scheme being 4/2/5/1 and for picks 14, 28, 42, 56, 70 and 84, the weft has one under portion of length 5, one under portion of length 4 one over portion of length 2 and one over portion of length 1 with a scheme of 5/2/4/1. For the construction of FIG. 3, as an example:

Warp 1: 15/1 Ne (for the base).

Warp 2: 4/1 Ne (for the over portions).

Weft: 15/1 Ne.

Warp density on the loom: 33.

Weft density on the loom: 22.

Reed number: 70/4/182 (5096 warp ends, reed length 1820 mm).

Fur length, i.e. the length of the warp long over portion (length 79 yarns), of this example is 36 mm with weaving report of FIG. 3.

FIG. 4 is a weaving report of an alternative embodiment of the fabric of the invention again representing the warp direction single front face fur design. FIG. 4 weaving report is a 12×101 construction that for reasons of clarity has been represented in two semi-reports. The construction of FIG. 4 is provided with a warp having a long (length 100) over portion and one short under portion (length 1) for warps numbered 1, 2, 4, 5, 7, 8, 10, and 11 with a scheme 100/1. For warps numbered 3, 6, 9 and 12, the construction of FIG. 4 is provided with warps having 51 over portions of length 1 and 50 under portions of length 1 with a scheme of 1/1.

In the scheme of FIG. 4, the weft has two long under portions (length 5) and two short over portions (length 1) with a scheme of 5/1/5/1 except for picks 9 and 23 which has two long under portions (of length 4) and two short over portions (length 2) with a scheme 4/2/4/2. Also for picks 13 and 17, the weft has two long under portions (of length 3), two short under portions (length 1) and four short over portions of length 1 with a scheme of 3/1/1/1/3/1/1/1.

FIG. 5 is a weaving report of still another embodiment of the fabric of the invention; again representing the warp direction single front face fur design. FIG. 5 weaving report is a 16×101 construction that for reasons of clarity has been represented in two semi-reports. The construction of FIG. 5 is provided with a warp having a long (length 100) over portion and one short under portion (length 1) for odd-numbered warps 1, 3, 5, 7, 9, 11, 13 and 15 with a scheme 100/1. For even-numbered warps 2, 4, 6, 8, 10, 12, 14 and 16, the construction of FIG. 5 is provided with warps having 25 over portions of length 3 and 35 under portions of length 1 with a scheme of 3/1.

The construction of FIG. 5 follows basically a twill scheme, with two weft under portions of length 7 and two weft over portions of length 1 with a scheme of 7/1/7/1 with the exception of pick 3 and 101 having each two under portions of length 3, two under portions of length 2, two over portions of length 2 and two over portions of length 1, with a scheme of 1/3/1/2/2/3/1/2/1.

FIG. 6 is a weaving report in the weft direction of another embodiment of the fabric of the invention representing weft direction on the single back side denim fur design. FIG. 6 weaving report is a 12×84 construction that for reasons of clarity has been represented in two semi-reports. The construction of FIG. 6 is provided with a weft having a long (length 79) under portion, two short under portions (length

1) and two short over portion (length 1) for odd-numbered picks 1, 3, 5, 7, 9, and 11 with a scheme 79/1/1/1/1.

For even-numbered picks 2, 4, 6, 8, 10 and 12, the construction of FIG. 6 is provided with wefts having 28 under portions of length 2 and 28 over portions of length 1 with a scheme of 2/1. The construction of FIG. 6 follows basically a twill scheme and is provided with a warp having two long (length 5) over portions and two short under portions (length 1) with a scheme of 5/1/5/1.

As exceptions, warps 3, 17, 31, 45, 59 and 73 show warps provided with two long over portions (respectively of length 4 and 5) and two short under portions (respectively of length 2 and 1) with a scheme of 4/1/5/2. Warps 5, 19, 33, 47, 61 and 75 are provided with two short over portions of length 2, a long over portion of length 5 and three under portions of length 1 with a scheme of 2/1/5/1/2/1b. Warps 15, 29, 43, 57 and 71 are provided with two long over portions (respectively of length 4 and 5) and two short under portions (respectively of length 2 and 1) with a scheme of 5/1/4/2.

FIG. 7 is a further weaving report in the weft direction of another embodiment of the fabric of the invention representing weft direction on the single back side denim fur design. FIG. 7 weaving report is a 12×84 construction that for reasons of clarity has been represented in two semi-reports.

The construction of FIG. 7 is provided with a weft having a long (length 83) under portion and one short over portion (length 1) for picks 1, 2, 4, 5, 7, 8, 10 and 11 with a scheme 83/1. For picks 3, 6, 9, 12 the construction of FIG. 7 is provided with wefts having 42 over portions of length 1 and 42 under portions of length 1 with a scheme of 1/1.

The construction of FIG. 7 follows basically a twill scheme and is provided with a warp having two long (length 5) over portions and two short under portions (length 1) with a scheme of 5/1/5/1. As exceptions, warps 64 and 76 show warps provided with two long over portions (length 4) and two short under portions (length 2) with a scheme of 4/2/4/2 and warps 68 and 72 show with two long over portions (length 3), two short over portions (length 1) and four short under portions (length 1) with a scheme of 3/1/1/3/1/1/1.

FIG. 8 weaving report is a 17×101 construction that for reasons of clarity has been represented in two semi-reports representing a weft direction single back denim fur design. The construction of FIG. 8 is provided with a weft having a long (length 100) under portion and one short over portion (length 1) for odd-numbered picks 3, 5, 7, 9, 11, 13, 15, and 17 with a scheme 100/1. For even-numbered picks 2, 4, 6, 8, 10, 12, 14 and 16 the construction of FIG. 8 is provided with wefts having 25 under portions of length 3 and 25 over portions of length 1 with a scheme of 3/1.

The construction of FIG. 8 follows basically a twill scheme and shows warps provided with two long over portions (respectively of length 7 and 8) and two short under portions (length 2 and 1) with a scheme of 7/1/8/1, with the exception of warps 1 which show a scheme of 3/2/1/3/2/2/1/3 and 99 which show a scheme of 4/1/2/2/3/1/2/2.

FIG. 9 is another weaving report in the weft direction of a further embodiment of the fabric of the invention representing weft direction on the front side denim fur design. FIG. 9 weaving report is a 12×84 construction that for reasons of clarity has been represented in two semi-reports.

The construction of FIG. 9 is provided with a weft having a long (length 79) over portion, two short over portions (length 1) and three short-under portions of (length 1) for odd-numbered picks 1, 3, 5, 7, 9 and 11 with a scheme of 79/1/1/1/1. For even-numbered picks 2, 4, 6, 8 and 10 the

weft is provided with 28 over portions of length 1 and 28 under portions of length 2 with a scheme of 2/1.

In the weaving report of FIG. 9, a twill pattern is repeated. In particular, the construction of FIG. 9 shows warps provided with four short over portions (of length 1), two long under portions (of length 3) and two short under portions (of length 1) with a scheme of 1/1/1/3/1/1/1/3.

As exceptions, in order to create a repeated twill pattern, warps 1, 15, 29, 43, 57 and 71 are provided with one over portion of length 2 and three over portions of length 1, one under portion of length 3, one under portion of length 2 and two under portions of length 2 with a scheme of 2/1/1/3/1/1/2.

Warps 17, 31, 45, 59 and 73 are provided with one over portion of length 2 and three over portions of length 1, one under portion of length 3, one under portion of length 2 and two under portions of length 1 with a scheme of 2/1/1/3//1/1/1/2 and warps 5, 19, 33, 47, 61 and 75 are provided with one over portion of length 3 and two over portions of length 1, two under portions of length 3 and one under portion of length 1 with a scheme of 3/3/1/1/1/3. Warp 2 has a scheme of 1/3/1/1/1/3/1/1.

FIG. 10 is still another weaving report of a further embodiment of the fabric of the invention. FIG. 10 weaving report is a 12×208 construction that for reasons of clarity has been represented in three portions. This fabric has warps doing over portions and under portions at the same time with different lengths of over/under portions in a same warp.

The construction of FIG. 10 is provided with a warp having a long (length 93) over portion, one shorter over portion of length 8, three short (binding) over portions of length 1, a long (length 92) under portion, one under portions of length 9 and three short under portions of length 1 for picks numbered 1, 4, 7 and 10 with a scheme of 1/1/9/1/93/1/1/8/1/92.

The construction of FIG. 10 is also provided with a warp having a long (length 89) over portion, one over portion of length 12, two short over portions of length 1, a long (length 88) under portion, one under portion of length 14, one under portion of length 2 and one short under portion of length 1 for picks numbered 2, 5, 8 and 11 with a scheme of 1/2/12/1/89/14/1/88.

The construction of FIG. 10 is also provided with a warp yarns, i.e. second warp yarns, having 104 short over portions of length 1, and 104 short under portions of length 1 for picks numbered 3, 6, 9 and 12 with a scheme of 1/1. The warp yarns are arranged to provide alternated second warp yarns and first warp yarns in a ratio 1/2, i.e. there are two first warp yarns for every second warp yarns.

The construction of FIG. 10 is also provided with a weft having two over portions of length 2, two over portions of length 1, two under portions of length 2 and two under portions of length 1 for odd-numbered wefts with a scheme of 1/1/2/2/1/1/2/2. For even-numbered wefts, the construction of FIG. 10 is provided with a weft having two over portions of length 2, two over portions of length 1, two under portions of length 2 and two under portions of length 1 with a scheme of 2/2/1/1/2/2/1/1.

For weft numbered 3, 16, 116, 107, the construction presents one over portion of length 5, one over portion of length 6, and two under portion of length 1, with a scheme of 6/1/5/1. For weft numbered 12 and 120 the construction presents two under portions of length 5, two over portions of length 2 and one over portion of length 1 with a scheme of 5/2/5/1.

FIG. 11 is another weaving report of a further embodiment of the fabric of the invention. FIG. 11 weaving report

is a 12×84 construction that for reasons of clarity has been represented in two semi-reports. The construction of FIG. 11 is designed in order to have both warp and weft yarns to create over portions.

5 In particular, pick 1 of the construction of FIG. 11 has eight over portions of length 5, four over portions of length 4, four over portions of length 2, four under portions of length 2 and twelve under portions of length 1 with a scheme of 4/2/5/1/4/2/5/1/5/2/4/1/5/1/5/1/2/1/2/1/5/1/5/1/2/1/2/1.

Pick 2 has two long over portions respectively of lengths 38 and 40, two short over portions of length 1 and four short under portions of length 1 with a scheme of 38/1/1/1/1/40/1. Pick 3 has eleven over portions of length 5, three over portions of length 4, three under portions of length 2 and eleven under portions of length 1 with a scheme of 5/1/4/2/5/1/5/1/5/2/4/1/5/1/5/1/4/2/5/1/5/1/5/1.

Pick 4 has two long over portions respectively of lengths 20 60 and 18, one over portion of length 1, one under portion of length 3 and two under portions of length 1 with a scheme of 60/3/1/1/18/1. Pick 5 has seven over portions of length 5, 15 15 two over portions of length 4, one over portion of length 3, seven under portions of length 2 and eight under portions of 20 length 1 with a scheme of 3/2/5/1/4/2/4/2/5/2/4/1/5/1/4/2/5/1/5/1/5/1/2/1/2/1/5/2/4/2.

Pick 6 has two long over portions of length 36 and length 30 42, two over portions of length 1, one under portion of length 2 and two under portions of length 1 with a scheme of 36/42/1/2/1/1. Pick 7 has ten over portions of length 5, 30 three over portions of length 4, two over portions of length 2, three under portions of length 2 and twelve under portions of length 1 with a scheme of 5/1/4/2/5/1/5/1/5/1/4/2/5/1/5/2/4/1/5/1/5/1/2/1/2/1/5/1.

Pick 8 has two over portion of length 25 and length 50, 35 one over portion of length 2, two over portions of length 1, one under portion of length 2 and two under portions of length 1 with a scheme of 75/2/1/1/1/2/1. Pick 9 has eight over portions of length 5, six over portions of length 4, six under portions of length 2 and eight under portions of length 1 with a scheme of 2/5/1/4/2/4/2/5/1/5/2/4/1/5/1/5/1/5/1/5/2/4/1/4/2/4.

Pick 10 has (two over portion of length 11 and length 64), 45 one over portion of length 2, two over portions of length 1, one under portion of length 2 and three under portions of length 1 with a scheme of 75/2/1/1/1/2/1. Pick 11 has nine over portions of length 5, four over portions of length 4, one under portion of length 3, six under portions of length 2 and eight under portions of length 1 with a scheme of 5/1/4/2/5/1/5/2/3/2/5/1/5/2/4/1/5/1/4/2/5/1. Pick 12 has two long over portions respectively of lengths 52 and 26, 50 two over portions of length 1 and four under portions of length 1 with a scheme of 52/1/26/1/1/1/1.

FIG. 12 is a photograph of an embodiment of the fabric 55 of the invention on the warp direction and FIG. 13 is photograph of the embodiment of the fabric of the invention of FIG. 12 after rinse wash. In particular, a fabric in a state similar to the fabric of the section of FIG. 1. In fact, after weaving, although the initial lengths of, e.g., first and second warp yarns, w1 and w2, are the same, due to the very different weaving report of said yarns the free-floating of the, e.g., over portions of first warps w1 are longer than the distance (on the fabric) between the start and the end of the said over portions. The difference is increased by the finishing treatment, so as to reach on average 10-50% difference in length to provide a curved and/or undulated aspect of the over portions.

## 11

FIG. 14 is a photograph of another embodiment of the fabric of the invention of FIG. 2 on the weft direction after finishing treatment and FIG. 15 is a photograph of the embodiment of the fabric of the invention after a cutting process. As visible, the cutting, i.e. the process of dividing the over (or under) portions in two parts, results in a furry appearance that may be also increased by additional mechanical treatments.

FIG. 16 is a flowchart of a method according to the invention. The method starts with the yarns (block 100) that are subjected to a weaving process (block 110), for example using a dobby loom or other similar textile machine. In particular, warp yarns and weft yarns are weaved following a pattern whereby the warp yarns are extending over a number of weft yarns and below a number of weft yarns to provide warp over portions in said front side and warp under portions in said back side and wherein the warp over portions have a length comprised between 8 and 3000 yarns, preferably 8 to 300 yarns. In an embodiment the overportions or underportions of the first warp yarns or of the first weft yarns have a discontinuity, i.e. are divided into two portions, e.g. obtained by laser cutting the first yarns. In this embodiment the two portions of the original over or under portions extend from the fabric at two locations that are spaced by a distance (e.g. measured in number of warps or wefts over which the over/underportion floats before being cut) corresponding to the original length of the over or underportions. In general, in an embodiment having discontinuous (i.e. cut or broken) over or under portions of the first yarns, the said portions may extend (i.e. float), when integral, for a length of 8 to 3000 warp or weft yarns. That is, in one embodiment, two warp portions produced by cutting the warp over portion have a combined length such that would extend past between 8 and 3000 weft yarns. Stated alternatively, the two portions of cut warp yarn extending from the fabric have a combined length such that extends past between 8 and 3000 weft yarns. In other embodiments, the warp over portions or warp under portions have a length such that extends past between 30 to 3000 weft yarns or between 40 to 3000 weft yarns. Stated alternatively, the two portions of cut warp yarn extending from the fabric have a combined length such that extends past between 30 and 3000 weft yarns or between 40 and 3000 weft yarns in the respective embodiments.

In some embodiments, the warp over portions extend over weft yarns so as to have a length comprised between 40 and 100 yarns. In a similar manner, instead of warp over portions, warp under portions can be provided. Warp over portions are preferred to impart the required furry appearance to the final fabric.

In an alternative embodiment, warp yarns and weft yarns are weaved following a pattern whereby the weft yarns are extending over a number of warp yarns and below a number of warp yarns to provide weft over portions in said front side and weft under portions in said back side. The weft over portions have a length comprised between 25 and 3000, preferably 25 to 300 yarns in some embodiments that is, the weft over portions extend past 25 to 3000 warp yarns in some embodiments and extend past 25 to 300 warp yarns in some embodiments. In some embodiments, the weft over portions have a length comprised between 40 and 100 yarns i.e. the weft over portions extend past 40 to 100 warp yarns. Thus, in some embodiments, the weft over portions have a length comprised between 40 and 3000 yarns, i.e., the weft over portions have a length that extends past 40-3000 warp yarns in some embodiments. In a similar manner, instead of weft over portions, weft under portions can be provided to

## 12

have a length comprised between 40 and 3000 yarns, i.e., the weft under portions have a length that extends past 40-3000 warp yarns. According to one embodiment, the fur look of the fabric is accomplished by the discontinuity formed by cutting the long weft over portions and the long weft under portions that include a length of 40 to 3000 yarns. Once cut to form the discontinuity, the long weft over or under portions of the first yarns, form two weft portions that each extend from the fabric base structure. The cutting of the weft under or over portions that have a length of between 40 and 3000 yarns prior to cutting, thus results in each of the cut weft over or under portions forming two weft portions having a combined length between 40 and 3000 yarns, that is, the two weft portions produced by cutting have a combined length such that would extend past between 40 and 3000 warp yarns. Stated alternatively, the two portions of cut weft yarn extending from the fabric have a combined length such that extends past between 40 and 3000 warp yarns.

The woven fabric is the subjected to a finishing process (block 120). According to an embodiment, then the finished fabric may be subjected to a cutting process (block 130). The cutting process can be performed with any suitable machine with a knife or laser or using any type of chemical application for cutting. In general, the cutting process is used to improve or increase the fur-like look of the final product. Cutting can be made in different ways by using different machines. Laser cutting can be used in particular after a laundry process (block 150). In a further alternative embodiment, after a laundry process (block 150) no cutting is performed (block 170).

After cutting, the fabric may be subjected to a laundry process (block 140). In an alternative embodiment, a laundry process (block 150) is performed before cutting. Then a cutting process is performed (block 160).

In general, the cutting process can be performed in a wide variety of ways, namely using:

- 1) Any cutting machine known in the art including a knife
- 2) Laser cutting
- 3) Ultrasonic fabric cutting machines
- 4) Any suitable chemical treatment

Concerning chemical treatments that can be used for the cutting process as described in the present invention, further details are provided here below.

Burn-out chemical agents can be used. Burn-out agents are strong acids as compounds which split off strong acids and which, in a subsequent heat treatment, destroy the cellulosic fibres. Heat treatment temperature can be 120-200 C°, preferably 140-180 C°. Suitable examples of burn-out agents are sulphuric acid and amino sulphonic acid, sodium bisulphate, aluminium sulphate, aluminium chloride, magnesium chloride, dibutylphthalenesulphonic acid and p-toluenesulphonic acid, methanesulphonic acid and sulphonic acids from among arenemonosulphonic or arenedisulphonic acids.

Further suitable burn-out agents are the alkali metal salts of sulphonic acids, particular the sodium or potassium salts in combination with sulphuric acid.

Preferable burn-out agents are sodium bisulphate, aluminium sulphate, p-toluenesulphonic acid, methane-sulphonic acid and alkylphthalene sulphonic acids possibly mixed with sulphuric acid.

The fabric is printed with the burn-out agent as customary in the form of a burn-out paste. Print can be full print or designed print.

The amount of burn-out agent to be used in the burn-out pastes increases with the cellulose content of the blend fabric.

## 13

Active burn out agents such as, for example, sodium bisulphite or hydrogensulphite may be 20-350 gr/kg, and preferably 50 to 250 gr/kg. These quantities are normally required to obtain acceptable burn-out style fabrics at the amounts of burn-out paste customarily used and to destroy cellulosic fibres.

Active burn-out agents, such as, sulphonated acids require as a rule burn-out agent concentrations in the burn-out pastes of 3 to 160 gr/kg, preferably to 40 to 140 gr/kg. As is usual the burn-out pastes in addition to the burn-out agents also contain water, thickeners and auxiliaries dispersing agent, wetting agent, carrier, glycerol). Examples of suitable thickeners are starch degradation products such as dextrin, non-ionic starch derivatives, such as British gum, types of gum, such as gum arabic, locust bean gum ether thickener and guar derivatives.

While at least one exemplary embodiment was disclosed in the foregoing summary and detailed description, it should be appreciated that a vast number of variations exist. The exemplary embodiments are only examples, and are not intended to limit the scope, applicability, or configuration in any way. Rather, the foregoing summary and detailed description will provide those skilled in the art with a convenient road map for implementing at least one exemplary embodiment, it being understood that various changes may be made in the function and arrangement of elements described in an exemplary embodiment without departing from the scope as set forth in the appended claims and their legal equivalents.

The invention claimed is:

1. A garment comprising a woven denim fabric that imitates natural fur, the denim fabric having warp yarns and weft yarns, said denim fabric having a front side and a back side,

said warp yarns and weft yarns being woven together in a weaving pattern, the weaving pattern comprising alternated first and second warp yarns and alternated first and second weft yarns, the weaving pattern of at least said second warp yarns and second weft yarns providing a base structure of the denim fabric, whereby said first warp yarns extend over said weft yarns in said front or back side of the denim fabric to provide warp over portions in said front side and/or warp under portions in said back side and

wherein at least some of the warp over portions and/or warp under portions extend over a length of between 30 and 3000 weft yarns, wherein only at least part of said over portions or under portions of said first warp yarns include a discontinuity,

wherein each said discontinuity comprises two portions of yarn extending from said denim fabric and having a combined length such that extends past between 30 and 3000 weft yarns; and

wherein said second warp yarns extend over only 1 to 4 warps.

2. The garment of claim 1, further comprising weft over portions and weft under portions, wherein at least some of the weft over portions and/or weft under portions extend over a length comprised between 40 and 400 warp yarns.

3. The garment of claim 1, wherein a first warp over portion of said warp over portions of said first warp yarns, or a first weft over portion and/or a first warp under portion of said warp under portions of said first warp yarns or a first weft under portion extend over a length in the range of 45 to 400 weft or warp yarns.

## 14

4. The garment of claim 1, wherein said warp over portions and/or said warp under portions have a count in the range from Ne 0.5 to Ne 40.

5. The garment of claim 4, wherein said second warp yarns have a count in the range from Ne 5 to Ne 100.

6. The garment according to claim 1, wherein at least part of said first warp yarns or first weft yarns are dyed or ring dyed.

7. The garment of claim 1, wherein each said discontinuity is on the front side of said garment.

8. The garment of claim 1 further comprising weft over portions and weft under portions, wherein said first warp yarns or weft yarns forming said over portions or under portions have a count in the range from Ne 2 to Ne 15.

9. The garment of claim 1, wherein the alternated first and second warp yarns are alternated such that a ratio of a number of first yarns:a number of second yarns is 3:1.

10. The garment of claim 1, wherein the alternated first and second warp yarns are alternated such that a ratio of a number of first yarns:a number of second yarns is 1:3.

11. The garment of claim 1, wherein at least some of the warp and/or weft yarns are elastic.

12. The garment of claim 1, wherein some of the warp over portions have a length ranging from 18 mm to 1400 mm.

13. The garment of claim 12, further comprising weft over or under portions having a length in the range from 8 mm to 110 mm.

14. The garment of claim 1, wherein the denim comprises said weft and warp yarns in a twill design, said warp over portions and/or said warp under portions have a count in the range from Ne 0.5 to Ne 40, and said second warp yarns have a count in the range from Ne 5 to Ne 100.

15. The garment of claim 1, wherein each said discontinuity comprises two portions of yarn extending from said denim fabric and having a combined length such that extends past between 30 and 450 weft yarns.

16. A method of preparing a garment with a fabric that imitates natural fur, said method comprising:

weaving warp yarns or weft yarns following a pattern providing alternated first and second warp yarns and alternated first and second weft yarns,

the weaving pattern of at least said second warp and weft yarns providing a base structure of the fabric,

whereby at least one of said first warp yarns and said first weft yarns extends over a number of weft or warp yarns and/or below a number of weft or warp yarns to provide warp or weft over portions in a front side and/or warp or weft under portions in a back side and

wherein only at least some of the warp over portions and/or warp under portions extend over a length of between 40 and 3000 weft yarns and at least some of the weft over portions and/or weft under portions extend over a length of between 40 and 400 warp yarns;

cutting at least some of said warp over portions or said warp under portions to produce a plurality of discontinuities, each said discontinuity associated with a cut one of said warp over portions or said warp under portions and comprising two portions of cut yarn extending from said fabric and having a combined length such that extends past between 40 and 3000 weft yarns; and

wherein said second warp yarns extend over only 1 to 4 warps.

**15**

17. The method of claim **16**, wherein the warp or weft over portions and/or the warp or weft under portions of said first yarns extend over a length comprised between 45 to 400 weft or warp yarns.

18. The method of claim **16**, wherein said cutting comprises cutting using ultrasonic fabric cutting machines or chemical treatment with burn-out agents.

19. The method of claim **10**, wherein some of the warp or weft over portions and/or the warp or weft under portions of said first yarns are whole.

20. The method of claim **16**, wherein said cutting comprises cutting with an ultrasonic fabric cutting machine.

21. The method of claim **16**, wherein said cutting comprises using a chemical treatment with burn-out agents, said burn-out agents comprising sodium bisulphite or aluminium sulphate.

22. The method of claim **16**, further comprising carrying out a laundry process prior to said cutting.

23. A garment comprising a woven fabric that imitates natural fur, the fabric having warp yarns and weft yarns, said fabric having a front side and a back side, said warp yarns and weft yarns being woven together in a weaving pattern, the weaving pattern comprising alternated first and second warp yarns and alternated first and second weft yarns, the weaving pattern of at least said second warp yarns and second weft yarns providing a base structure of the fabric,

5

10

15

20

25

**16**

whereby said first warp yarns extend over a number of said weft yarns at least on said front side of the fabric to provide warp over portions in said front side and wherein at least some of the warp over portions extend over a length of between 40 and 3000 weft yarns, wherein only at least some of said warp over portions of said first warp yarns include a discontinuity, wherein each of said over portions that include a discontinuity are formed of two portions of yarn extending from said fabric and having a combined length such that extends past between 40 and 3000 weft yarns; and wherein said second warp yarns extend over only 1 to 4 yarns.

24. The garment of claim **23**, wherein the alternated first and second warp yarns are alternated in such that a ratio of a number of first yarns:a number of second yarns is 1:3.

25. The garment of claim **23**, wherein some of the warp over portions have a length ranging from 18 mm to 1400 mm.

26. The garment of claim **23**, wherein at least some of the warp and/or weft yarns are elastic.

27. The garment of claim **23**, wherein said second warp yarns have a count in the range from Ne 5 to Ne 100 and said warp over portions and/or said warp under portions have a count in the range from Ne 0.5 to Ne 40.

\* \* \* \* \*